

1

3,537,999

LUBRICANTS CONTAINING BENZOTHIADIAZOLE  
Brian R. Kennedy, San Rafael, Calif., assignor to Chevron Research Company, San Francisco, Calif., a corporation of Delaware

No Drawing. Filed Dec. 11, 1968, Ser. No. 783,142

Int. Cl. C10m 1/38, 3/32

U.S. Cl. 252—47.5

5 Claims

## ABSTRACT OF THE DISCLOSURE

Lubricating oil compositions provided extreme pressure and wear-inhibiting properties by minor amounts of 1,2,3-benzothiadiazoles.

## BACKGROUND OF THE INVENTION

### Field of the invention

In lubricating oils, particularly ash-free or low ash lubricating oils, used in internal combustion engines, it is common to add antioxidant and antiwear agents. It is, in particular, usual to add metal salts, particularly zinc salts, of various phosphorodithioic acid esters for this purpose. However, there have been continual efforts to reduce the amount of metal in lubricating oils, as these metals in ionic form frequently enhance deposit formation during service. It has thus been wished to provide antiwear and antioxidant materials which do not provide undesirable metal ions.

It has been further desired to provide lubricants which possess extreme pressure characteristics, e.g., to reduce wear on bearings, etc. when they are subjected to the application of large forces. This has been accomplished with the use of various additives, particularly chlorine substituted organic compounds such as chlorinated waxes.

### Description of the prior art

Many patents are issued on the use of nitrogen and sulfur containing heterocycles in lubricating oil. U.S. Pat. 2,218,283 discloses mercaptobenzodiazoles in lubricating oils. Likewise, U.S. Pat. 2,318,629 discloses organic sulfur compounds in lubricating oils. Also included are those compounds which also contain a nitrogen atom such as thiazole and thiazene derivatives. U.S. Pat. 2,154,096 discloses monovalent radical substituted thiazenes and thiazoles as corrosion inhibitors with hard metal alloy bearings.

## SUMMARY OF THE INVENTION

Lubricating compositions are provided comprising a major proportion of an oil of lubricating viscosity and a minor proportion, sufficient to provide wear, corrosion inhibiting and extreme pressure properties, of 1,2,3-benzothiadiazole or its chlorinated analogs. Thus the additives of this invention are the following formula:



in which X is chlorine and n=0-4.

## DESCRIPTION OF THE PREFERRED EMBODIMENTS

1,2,3-benzothiadiazole is well known as a dye intermediate. Its preparation is, therefore, well known in the

2

art. The compound can be produced by the reaction of 2-aminothiophenol with nitrous acid or with nitrosyl-sulfuric acid. A representative chlorine-substituted material may be prepared by the reaction of 2,2'-dithio-bis-(5-chloroaniline), a commercially available material with nitrosyl sulfuric acid.

In general, in reacting with nitrosyl sulfuric acid, the temperature of the reaction mixture is kept low, preferably not above 5° C.

10 The lubricating oils in which the benzothiadiazoles are used may be derived from natural or synthetic sources. Lubricating oils generally have viscosities of from about 35 to 50,000 Saybolt Universal Seconds (SUS) at 100° F. Among natural hydrocarbonaceous oils are paraffinic base, naphthenic base, asphaltic base and mixed base oils. Illustrative synthetic hydrocarbonaceous oils are polymers of various olefins, generally of from 2 to 8 carbon atoms and alkylated aromatic hydrocarbons.

15 The benzothiadiazoles are preferably compounded with from 1 to 15 weight percent of a polyalkylene polyamine lubricating oil detergent. These detergents are described in U.S. Pats. 3,219,666 and 3,202,678. The polyalkylene polyamines will generally have from 2 to 6 nitrogen atoms and alkylene groups of from 2 to 3 carbon atoms. Bonded to the alkylene polyamines will generally be from 1 to 2 oil soluble aliphatic hydrocarbon groups, usually a polymer of olefins of from 3 to 4 carbon atoms (propene and isobutylene). The hydrocarbon groups are bonded to the alkylene polyamine directly to nitrogen or through a nonoxocarbonyl group such as formyl or succinoyl. The aliphatic hydrocarbon group will generally be of from 30 to 200 carbon atoms, more usually of from 50 to 150 carbon atoms.

20 Other additives may also be present, such as antirust agents, corrosion inhibitors, other detergents, additional oxidation inhibitors, oiliness agents, etc.

25 The 1,2,3-benzothiadiazoles will generally be present in from 0.1 to 10.0% by weight of lubricating oil compositions, more usually from about 0.5 to 5.0% by weight. The other additives will generally be present individually in from about 0.01 to 15 weight percent, more usually from about 0.05 to 10 weight percent. The alkylene polyamine detergent will usually be present in from 2 to 15 weight percent.

30 The following examples are offered by way of illustration and not by way of limitation.

35 Example I.—Preparation of 1,2,3-benzothiadiazole: 60 g. (0.44 moles) of 2-aminothiophenol was mixed with 50 ml. of water in a 500 ml. flask. A solution of 25 ml.

40 of sulfuric acid in 125 ml. H<sub>2</sub>O was cooled to 0° C. and added slowly with stirring to the reaction flask, the contents of which were likewise cooled to 0±2° C. An ice cold solution of sodium nitrite (34 g. in 50 ml. H<sub>2</sub>O) was added dropwise as a slurry to the reaction flask over a period of four hours while the temperature of the mixture was maintained at 2±2° C. The solid material which precipitated from the reaction mixture was filtered from the mixture and steam distilled. The product was then dried in a desiccator over NaOH.

45 Example II.—Preparation of 6-chloro-1,2,3-benzothiadiazole: To 197 cc. of concentrated H<sub>2</sub>SO<sub>4</sub> cooled to 0° C. was slowly added 28.4 g. of sodium nitrite. The mixture was stirred for 15 min., heated to 70° C. and cooled to -10° C.

50 50.0 g. of 2,2'-dithio-bis-(5-chloroaniline) was dissolved in 134 ml. of concentrated H<sub>2</sub>SO<sub>4</sub> at room temperature with stirring. The mixture was then cooled to 0° C.

55 The second solution was added dropwise to the first with stirring over a period of 30 min. The mixture was then allowed to stand for 30 minutes and then poured into a liter of mixed ice and water. The mixture foamed and

emitted a brown vapor. It was allowed to stand over the weekend.

The solids were filtered from the mixture, dissolved in ether, and washed twice with water. The ether solution was dried with sodium sulfate and stripped, the residue being redissolved in toluene, from which it was recrystallized and then dissolved in mixed hexane, dried and stripped. The yield was 14.6 g. of a brownish solid having a melting range of 102.5–104° C. This material was then dissolved and recrystallized from an ethanol water mixture.

The residues were collected, stripped and chromatographed over silica gel with mixed hexanes and recrystallized from ethanol water mixture yielding 11 g. more for a total yield of 21 g. of 6-chloro-1,2,3-benzothiadiazole.

In order to demonstrate the excellent effectiveness of the benzothiadiazoles utilized in the lubricating oils of this invention in imparting EP and antiwear properties to lubes, a number of industry-recognized tests were performed.

To demonstrate the effectiveness of the lubricating oils under extreme pressure conditions, the oils were tested in the Falex Shear Test, results of which may be found in Table I following. The results are reported as load at failure in pounds.

TABLE I

| Formulation:                                    | Load at failure, lbs. |
|-------------------------------------------------|-----------------------|
| Base oil <sup>1</sup>                           | 850                   |
| Base oil + 0.5% 1,2,3-benzothiadiazole          | 1375                  |
| Base oil + 1.0% 1,2,3-benzothiadiazole          | 1700                  |
| Base oil + 2.5% 1,2,3-benzothiadiazole          | 2780                  |
| Base oil + 1.0% 4-chloro-1,2,3-benzothiadiazole | 1055                  |
| Base oil + 2.0% 4-chloro-1,2,3-benzothiadiazole | 1985                  |

<sup>1</sup> 480 neutral oil + 5 weight percent polyisobutylene succinimide of tetraethylene pentamine (polyisobutylene ~1000 mol. wt.) and 0.1 weight percent terephthalic acid (corrosion inhibitor).

These data show the effectiveness of 1,2,3-benzothiadiazole in increasing load to failure, by a factor of over 3:1 compared to the base oil alone, when the additive is employed at 2.5% concentration.

In order to demonstrate the degree of protection provided to copper and lead bearing material by the compositions of this invention, copper and lead strips were immersed in oil formulation employing the same base oil and detergent additive as in the Falex Test. The immersion was continued at a temperature of 340° F. for 20 hours. During the heating period, the oil is vigorously stirred. At the end of the test period, the strips are removed and weight loss is determined. The copper strip is washed with KCN to remove copper salts which may

form on the surface. The results may be found in the following table:

TABLE II.—COPPER-LEAD STRIP CORROSION TEST

| Type                          | Additive | Concen-<br>tration,<br>wt.<br>percent | Weight loss, mg. |                     |                    |
|-------------------------------|----------|---------------------------------------|------------------|---------------------|--------------------|
|                               |          |                                       | Pb               | Cu<br>Before<br>KCN | Cu<br>After<br>KCN |
| (Base oil).....               |          |                                       | 928              | 12.4                | 15.6               |
| 1, 2, 3-benzothiadiazole..... |          | 0.2<br>1.0                            | 855<br>557       | 22.2<br>9.5         | 25.3<br>15.1       |

It may be seen from these data that 1,2,3-benzothiadiazole is effective in reducing copper and lead corrosion, while as previously noted, it is very effective in increasing the extreme pressure resistance.

I claim:

1. Lubricating oil composition containing a hydrocarbon lubricating oil and in an amount sufficient to provide wear and corrosion inhibiting and extreme pressure properties an additive which is a benzothiadiazole or chlorinated benzothiadiazole of the formula:



in which X is chlorine and  $n$  is 0–4.

2. A lubricating oil composition according to claim 1 in which  $n$  is 0.

3. A lubricating oil composition according to claim 1 in which the extreme pressure additive is 1,2,3-benzothiadiazole.

4. A lubricating oil composition according to claim 1 having from 2-15 weight percent of an alkylene polyamine of from 2 to 6 nitrogen atoms, wherein the alkylene groups are from 2 to 3 carbon atoms, having bonded to nitrogen of from 1-2 oil soluble aliphatic hydrocarbon groups of from 30 to 200 carbon atoms, wherein said aliphatic hydrocarbon groups are bonded to nitrogen either directly or through a nonoxocarbonyl group.

5. A lubricating oil composition according to claim 2 where the additive is present in the amount of from about 0.5 to 5.0 percent by weight.

## References Cited

UNITED STATES PATENTS

2,154,097 4/1939 Loane ----- 252-47.5  
2,218,283 10/1940 Fuller ----- 252-47

## FOREIGN PATENTS

972,388 7/1959 Germany.

55 DANIEL E. WYMAN, Primary Examiner  
J. M. HICKEY, Assistant Examiner

U.S. Cl. X.R.